

## UNITED STATES PATENT OFFICE.

CHARLES E. LEHR, OF BETHLEHEM, PENNSYLVANIA, ASSIGNOR TO BETHLEHEM STEEL COMPANY.

## MOLD COMPOUND.

No Drawing.

Application filed May 27, 1925. Serial No. 33,287.

*To all whom it may concern:*

Be it known that I, CHARLES E. LEHR, a citizen of the United States, and resident of Bethlehem, Lehigh County, State of Pennsylvania, have invented certain new and useful Improvements in Mold Compounds; of which the following is a specification.

This invention relates to a mold or core material. The object of the invention is to revivify foundry sand by the addition of comminuted slag such as may be procured by the operation of a blast furnace, open hearth furnace or the like. The slag is crushed or ground into fine particles by any suitable apparatus and mixed with the inert sand together with a small quantity of fire clay, the latter ingredient constituting a binding medium so that the compound may be formed into various shapes as required in foundry operations.

The invention contemplates a compound for forming molds having a high degree of permeability to the passage of gases evolved in the casting operation and, furthermore, provides a material having high refractory properties, which prevent the material from burning fast to the castings and avoids the formation of scabs thereon.

I have found that a mixture consisting of approximately four parts comminuted slag and one part silica sand with a small percentage of fire clay provides a very desirable material for making molds or cores for the casting of metals.

While the principal object of my invention is to provide a compound for revivifying sands usually employed in foundry practice, nevertheless, it should be understood that my invention further contemplates the use of new sand as one of the constituents of my mixture.

It is customary in foundry operations, particularly steel foundry practice, to use 40 to 60% of new sand incorporated with old sand when forming molds, due to sand becoming inert by the burning out of the vegetable matter and the fusing of the low grade fire clay which it contains.

In accordance with my invention, I use comminuted slag. This ingredient is not

only cheap, being ordinarily a waste by-product of blast or open hearth furnace operation, but it also gives a degree of stability to the mold or core mixture, the latter result being due to the fibrous nature or characteristic of the slag.

As already pointed out, I prefer to prepare a mixture consisting of approximately four parts of comminuted slag and one part of sand containing a sufficient amount of argillaceous material. If the sand is new, there may be sufficient vegetable and clay matter to form a binder; however, with use, sand becomes inert, the vegetable matter burning out and the clay fusing, and, with old sand, I add a small amount of fire clay.

From the foregoing, it will be apparent that I have provided a mixture which greatly reduces the requirements for new sand for the reason the revivifying effect of my comminuted slag and fine clay additions permits of sand being used over and over again. Another advantageous feature is opening up a new field of use for a waste product, namely, slag; and owing to the abundance of slag, the cost of foundry operations may be greatly reduced. In addition to the economic advantages just pointed out, my composition is advantageous from the physical points of view of stability, or permeability for evolved gases, and of refractoriness.

I have stated above a proportion of the ingredients which provides a mixture suitable for a molding material, but I desire to have it understood that the proportions specified are merely given in their illustrative and not in their limiting sense.

What I claim as new and desire to secure by Letters Patent is:—

1. A compound suitable for forming foundry molds comprising a comminuted slag, foundry sand and fire clay.
2. A compound suitable for forming foundry molds comprising comminuted slag and silica sand.
3. A compound suitable for forming foundry molds comprising comminuted slag, inert foundry sand and fire clay.
4. A compound suitable for forming

foundry molds comprising comminuted foundry molds comprising about four parts metallurgical slag, silica sand and fire clay.

5. A compound suitable for forming foundry molds comprising about four parts comminuted slag, and about one part foundry sand and a small percentage of fire clay. <sup>10</sup> In testimony whereof I hereunto affix my signature this 22nd day of May, 1925.

6. A compound suitable for forming

CHARLES E. LEHR.